

Nov. 10, 1925.

1,561,168

W. V. D. KELLEY ET AL

COLOR PHOTOGRAPHY

Filed Feb. 5, 1924



INVENTOR

William V. D. Kelley  
Dominick Tronolone  
BY

Lyman E. Dodge  
ATTORNEY

## UNITED STATES PATENT OFFICE.

WILLIAM V. D. KELLEY, OF JERSEY CITY, AND DOMINICK TRONOLONE, OF FORT LEE, NEW JERSEY, ASSIGNEES TO KELLEY COLOR LABORATORY, INC., OF PALISADE, NEW JERSEY, A CORPORATION OF NEW JERSEY.

## COLOR PHOTOGRAPHY.

Application filed February 5, 1924. Serial No. 690,722.

To all whom it may concern:

Be it known that we, WILLIAM V. D. KELLEY, a citizen of the United States, and a resident of the city of Jersey City, county 5 of Hudson, State of New Jersey, and DOMINICK TRONOLONE, a citizen of the United States, and a resident of the town of Fort Lee, county of Bergen, and State of New Jersey, have invented a new and useful Im- 10 provement in Color Photography, of which the following is a specification.

This invention relates to color-photography and particularly has reference to the production of a plurality of colored registered images in a single coating on a transparent carrier.

Heretofore quite a few processes have been proposed for forming what is known as a color-photograph, that is, a photograph 20 which exhibits an image of a subject wherein a color appears in kind and position corresponding to the coloring of the subject.

For making colored photographic motion picture film it has heretofore been proposed 25 to form two registered superimposed images in the same picture space, one being formed of one color and the other being formed of a substantially complementary color. It has heretofore been proposed to secure one of the 30 colors by a toning process and the other by a dyeing process or both by a dyeing process.

The principal object of applicants' invention is to provide a process by which at least 35 two substantially complementary colored superimposed images in the same picture space, in a single coating on one side only of a carrier may be obtained by methods which involve the toning with metallic salts of two images without degradation of either.

Other objects and advantages will appear 40 as the description of a particular manipulation involving the novel features of applicants' invention progresses and the novel features will be particularly pointed out in the appended claims.

In describing the invention in detail and the particular physical product selected to illustrate the invention, reference is had to the accompanying drawing wherein we have 45 illustrated a particular preferred physical product resulting from the practice of our invention, and wherein like characters of

reference designate corresponding parts throughout the several views, and in which:

Figure 1 is a schematic representation of 55 a colored object; Fig. 2, is a representation of the ordinary and well known red color selection negative of the object Fig. 1; Fig. 3, is a representation of the ordinary and well known blue-green color selection negative 60 of the object, Fig. 1; Fig. 4, is a schematic representation of a black and white print made from the negative Fig. 2; Fig. 5, is a schematic representation of a black and 65 white print made from the negative Fig. 3; Fig. 6, illustrates the print, Fig. 4 colored; Fig. 7, illustrates the print Fig. 5 colored; Fig. 8, illustrates the combination of colored prints, Figs. 6 and 7.

In the drawing Figs. 4 and 5 are really 70 representations of the same, say, film, one Fig. 4 after a print from the red-orange negative Fig. 2, the other, Fig. 5, after printing from the blue-green negative. Fig. 3 and Figs. 6 and 7 are of course consequently 75 representations of the same, say, film, illustrating different operations thereon. Fig. 8 is also a representation of the same single film with a single emulsion coating thereon, 80 illustrating the combined effect of the different operations.

In order to carry out applicants' process it will be necessary to secure two images one representative of one color in a subject and the other representative of a substantially complementary color of the subject. These images of course must be suitable to be used 85 as negatives and in the further description of this process will be referred to as negatives. One will be designated the blue-green negative and the other the red negative. There are many ways of securing these negatives well known to those skilled 90 in this art and as applicants' process does not depend upon the particular methods used for securing the negatives no particular manner of securing them will be described and pointed out. The red negative in the drawing is illustrated by Fig. 2. The blue-green negative by Fig. 3.

Having secured the negative, one is placed in contact with the back of a transparent support carrying a single emulsion coating. If motion pictures are being dealt with, then 100

the negative would be placed in contact with the celluloid, that is, in contact with the uncoated side of the film and further, ordinary motion picture stock film would be used it 5 being unnecessary to use any dye in the emulsion to act as a light retardant. The negative having been placed in contact with the back of the film a printing light is then allowed to shine therethrough and a latent 10 image formed in the emulsion coating. In thus forming a latent image in the emulsion coating care is taken to so regulate the intensity of the printing light and the time of printing so that if possible the light sensitive 15 material in the emulsion which will be acted upon, will be substantially only that positioned in substantially the lower thickness of the emulsion coating.

After the printing with one negative 20 through the back of the carrier the latent image is developed for about three minutes. The particular developing bath considered by applicants to be most efficacious in enabling them to secure the desired result is 25 neutral or acid and would be made up as follows: Diamidophenol 5 g., sodium sulphite 30 g., potassium bromide .94 g., potassium iodide 10% solution 1.2 c. c., water 1 l.

After developing, the print should be 30 washed for 5 minutes, resulting in the print Fig. 4, then if the image is to be formed as a blue-green image, the print should be placed in what we term the color-forming bath. A satisfactory color-forming bath to 35 develop a blue-green in the image is formed as follows: Oxalic acid 5 g., vanadium oxalate 10% solution 15 c. c., ferric and ammonium oxalate 14 g., potassium ferricyanide 5 g., water 1 l.

40 The print should be allowed to remain in the blue-green color forming bath for 15 minutes and then washed for five minutes.

After the print has been washed it should be cleared. The applicants allow the clearing 45 bath to act for ten minutes and find that a suitable clearing bath would be as follows: ammonium bromide 12 g., potassium bichromate 12 g., water 2 l.

After the print has been cleared it should 50 be washed for ten minutes and dried. This drying must of course take place in the dark, or in a room illuminated by a light having no effect upon the light sensitive material in the emulsion, that is, in most cases with 55 a ruby light. After drying the finished toned print would be illustrated by Fig. 6.

After the print has been dried a second latent image is then to be formed in the emulsion coating. This second latent image 60 is to be formed by printing from the other negative by placing the same in contact with the emulsion and allowing a printing light to shine therethrough. The intensity of the printing light and the time of printing will 65 be preferably so regulated that the color

image formed by further manipulation resulting will be substantially complementary to the first color formed.

After the latent image is formed in the emulsion it is placed in the developing bath 70 hereinbefore described and developed for three minutes, after which it is washed for five minutes and fixed in sodium thiosulfate 600 g., water 1 l. and then washed for fifteen minutes. The effect of this second 75 printing and developing, disregarding the first formed blue-green image would be illustrated by Fig. 5.

The film now containing a blue-green 80 image and a reduced black silver image is placed in the red color forming bath. A red-orange color forming bath found suitable and preferred by the applicants would be formed as follows: uranium nitrate 9 g., potassium oxalate 4 g., hydrochloric acid 8 c. c., potassium ferricyanide 3.5 g., water 1 l.

The developed image would be allowed to remain in the red-orange color forming bath for five minutes and then washed for five minutes. The result of the red-orange color 90 forming bath would be illustrated by Fig. 7 disregarding the blue-green toning.

After the print has been last washed it would be fixed for five minutes in a bath 95 formed as follows: sodium thiosulfate 600 g., potassium metabisulphite 60 g., water 1 l.

After fixing, the print would be washed for ten minutes and then dried, thus completing the formation of the color photograph. That is, a transparent carrier having a coating on one side only and in that coating in the same picture area two, registered super-imposed, substantially complementary colored images. The completed 100 print toned blue-green and red-orange would be illustrated by Fig. 8.

Although applicants have illustrated the principle of their invention by describing the steps of a novel process which results in a novel product, nevertheless, it is to be understood that the particular manipulation described and the product formed does not exhaust the possible expressions of applicants' process and the tangible products to 110 be thereby produced.

What we claim is new and desire to secure by Letters Patent of the United States is:

1. A photographic process which consists in forming a latent image in a colloid layer, developing in neutral or acid diamidophenol toning with an iron salt and after clearing with a bath of ammonium bromide and potassium bichromate in water solution forming an image toned with an uranium salt 120 in the same colloid layer in registry there- 125 with.

2. A photographic process which consists in forming a latent image in a colloid layer developing in diamidophenol toning with an 130

iron salt and after clearing with a bath of ammonium bromide and potassium bichromate in water solution forming a second latent image in the same colloid layer, developing in diamidophenol and coloring.

3. A step in a photographic process which consists in forming an image in a sensitized colloid layer, toning said image and clearing with a bath of ammonium bromide and potassium bichromate in water solution.

4. A photographic process which consists in forming an image in a sensitized colloid layer, toning said image and clearing with a bath of ammonium bromide and potassium bichromate in water solution and thereafter forming and toning another registering image in the same colloid layer.

5. A photographic process which consists in printing two registered images in the same colloid layer and toning the same which includes the intermediate step of clearing with a bath of ammonium bromide and bichromate in water solution.

6. A photographic process which consists in forming an image toned with an iron salt in a colloid layer and after clearing with a bath of ammonium bromide and potassium bichromate in water solution forming an image toned with an uranium salt in the same colloid layer in register therewith.

7. The process which consists in first forming a silver image in a colloid layer, then toning that image substantially a blue-green, then forming another silver image in the same colloid layer and toning that image substantially a red orange, without affecting the color of the first image.

8. A photographic process comprising imprinting a negative image of an object from which certain color sensations have been omitted, upon light transmittive sensitized material, developing, washing and toning said image substantially a blue-green, clearing with a bath containing ammonium bromide and potassium bichromate in water solution, washing, drying and imprinting a second image of the same object, from which other color sensations have been omitted,

upon said material in registry with the first image imprinted thereon, developing said second image, washing in sodium thiosulfate and washing, then toning said second image a substantially red-orange by immersion in a bath containing uranium nitrate, potassium oxalate, hydrochloric acid and potassium ferricyanide in water solution, washing, fixing, washing and drying.

9. A photographic process in which by means of perforations in the carrier of a single light-sensitive emulsion two registered images are obtained, the first being printed, developed, converted to a salt of iron and bathed in a bath containing bromide and bichromate and dried without fixing, the second image being printed developed, fixed and converted to a salt of a metal giving a color tone complementary to the first.

10. The production in a colloid layer of silver print which is converted to a salt of iron then bathed in a bath containing bichromate and bromide, dried and a second silver print produced in registry with the first and the latter converted to a salt of uranium without affecting the color of the first image.

11. The production of two silver images in registry in the same colloid layer both independently developed in a diamidophenol developer, the first being converted to a salt of iron followed by immersion in a bath containing bichromate and bromide and after drying, printing and developing the second image and converting the latter to a salt of uranium.

12. The method of producing two images in the same colloid layer and converting each to a salt of a metal of different color each image being independently developed in a diamidophenol developer with an immersion in a bath containing a bromide and a bichromate after the first conversion and before the second development.

WILLIAM V. D. KELLEY.  
DOMINICK TRONOLONE.